

Patented Sept. 9, 1924.

1,508,083

# UNITED STATES PATENT OFFICE.

FRANK E. CLARK, OF NEW YORK, N. Y.

## MANUFACTURE OF STEEL.

No Drawing.

Application filed December 16, 1920. Serial No. 431,294.

To all whom it may concern:

Be it known that I, FRANK E. CLARK, a citizen of the United States, and resident of the city, county, and State of New York, <sup>5</sup> have invented certain new and useful Improvements in the Manufacture of Steel, of which the following is a specification.

My invention aims to provide a process of making steel and particularly chromium <sup>10</sup> steel and steel alloys by which such steel or steel alloys can be produced of great purity.

The process is performed in a basic lined furnace, preferably an electric furnace of <sup>15</sup> the Heroult arc type. A thorough deoxidation of the bath is secured by the use of a highly siliceous slag, this stage of the process being followed by the use of a slag lower in silica.

<sup>20</sup> A specific example of the process is as follows.—An ordinary cold charge, consisting generally of steel scrap, is put into a basic electric furnace and there melted under the usual basic oxidizing slag to de-phosphorize it. Such a slag, for example, comprises lime 50 to 60%, iron oxid 15 to 20%, and the balance magnesia, alumina and silica in unimportant proportions. The use <sup>25</sup> of this slag, while it serves to remove phosphorous, leaves the bath with a certain percentage of oxides in it which are objectionable particularly in the making of chromium steel and similar steels. These steels often contain defects caused primarily by <sup>30</sup> oxides of chromium or other alloying metal; which oxides are reduced only with great difficulty in the bath. The next step of the process, therefore, is directed to the thorough deoxidation of the bath.

<sup>40</sup> When the dephosphorization has been completed or carried to the desired extent, this first slag is removed and replaced by a highly siliceous slag, the principal purpose of which is to thoroughly deoxidize the <sup>45</sup> bath. Such a slag, for example, may contain 35 to 55% silica ( $SiO_2$ ) with the balance chiefly lime and with small quantities of magnesia and alumina. Under this slag the temperature of the bath should be increased, say from 1525 degrees centigrade <sup>50</sup> to above 1575 degrees and repeated layers of coke dust should be added on the slag until the deoxidation is substantially complete. The total quantity of coke dust will <sup>55</sup> probably average fifteen pounds to the ton of steel and in special cases may run up

to fifty pounds. The carbon in the added coke dust and in the bath reacts with the silica of the slag, reducing silicon therefrom, and the latter serves to deoxidize the <sup>60</sup> bath. The quantity of silicon reduced from the slag varies with the quantity of silica present in the slag. The time required for the reduction of the silicon is shortened as <sup>65</sup> larger quantities of silica are used in the slag. A certain percentage of silicon is required in the finished steel, about 0.20% in ordinary chromium steel. The percentage of silica in the slag and the length of time <sup>70</sup> this stage of the process should be such as to thoroughly deoxidize the bath and in addition to yield the silicon content required in the steel.

The operation with high siliceous slag <sup>75</sup> being completed, this slag is removed from the furnace and substituted by what I call a finishing slag, the principal function of which is to remove sulphur and to allow the impurities in the steel to rise to the surface under practically dead melting conditions. The finishing slag may be an ordinary basic slag, containing up to 25% silica with the balance essentially lime. The smaller the percentage of silica in this <sup>80</sup> finishing slag, the greater the sulphur-carrying capacity of the slag. A good example will be a slag containing about 10% silica. The presence of silica in reducing slags decreases the sulphur-carrying capacity but is <sup>85</sup> of material advantage in deoxidizing. By <sup>90</sup> my process I first use the slag best adapted for deoxidizing, and follow this by the slag best adapted for reducing the sulphur content of the bath.

<sup>95</sup> In my process the highly siliceous slag does not come into contact with the basic hearth except at the slag line, and, therefore, does not substantially scorch the hearth. It would be disadvantageous to use such a slag to finish the heat because when the heat is poured or tapped a portion of the slag settles over the entire hearth and would quickly cut it out. By removing this slag from the bath and finishing the metal under a highly basic slag, I secure the advantage of the high silica slag without serious injury to the furnace.

The process is applicable not only to making steel from cold scrap, but also to the refining of a molten charge such as molten Bessemer steel or molten acid or basic open hearth steel.

Where it is not necessary to remove phosphorous first from the bath, as in treating basic open hearth steel which has already been sufficiently dephosphorized, the basic 5 oxidizing slag above referred to is not necessary, and the process may be commenced with the highly siliceous slag added immediately after the metal is poured into the furnace.

10 In making the alloy steels referred to it is customary to add the alloying metal to the bath after dephosphorizing. For example, ferro-chrome is added to a dephosphorized steel bath to produce chromium steel analyzing usually 1% or more of chromium. In such addition, under the old practice, oxides of chromium are produced when the ferro-chrome is added and are reduced with great difficulty, or if not reduced are the cause of defects in the steel. According to my process, the alloying metal is added 15 after the highly siliceous slag has been used to remove the oxygen left in the bath by the dephosphorizing operation, and removal of such slag.

20 The principal function of the silica in the finishing slag is to increase its fluidity; and it may be replaced in whole or in part by fluorspar and other materials which are known to accomplish the same purpose.

25 Though I have described with great particularity of detail certain specific processes embodying my invention, yet it is not to be understood therefrom that the invention is restricted to the specific embodiments de-

scribed. Various modifications thereof may be made by those skilled in the art without departing from the invention as defined in the following claims.

What I claim is:

1. In the making of steel the process which comprises holding it molten on a basic hearth under a highly siliceous deoxidizing slag and replacing said deoxidizing slag by a slag lower in silica. 40

2. In the making of steel the process which comprises holding it molten on a basic hearth under an oxidizing slag for removal of phosphorous, replacing said deoxidizing slag by a highly siliceous deoxidizing slag and finally by a slag lower in silica. 45

3. In the making of alloy steel the process which comprises, first, holding the steel molten under a highly siliceous deoxidizing 50 slag, second, removing said deoxidizing slag, third, adding the alloying ingredient and fourth, replacing said deoxidizing slag by a slag lower in silica.

4. In the making of alloy steel the process which comprises holding the steel molten on a basic hearth under a highly siliceous deoxidizing slag, adding the alloying ingredient after the use of said deoxidizing slag, and replacing said deoxidizing slag by a 55 slag lower in silica. 60

In witness whereof, I have hereunto signed my name.

FRANK E. CLARK.